

Patented May 30, 1933

1,911,307

# UNITED STATES PATENT OFFICE

ALAN A. CLAFLIN, OF WINCHESTER, MASSACHUSETTS, ASSIGNOR TO NIACET CHEMICALS CORPORATION, A CORPORATION OF NEW YORK

## MORDANTING ASSISTANT AND PROCESS FOR USING THE SAME

No Drawing.

Application filed February 18, 1931. Serial No. 516,846.

This invention relates to mordanting textile fibers of animal origin for the purpose of fixing dyes therein and to a new assistant for mordanting operations. My invention especially concerns the use of aldol (CH<sub>3</sub>.CHOH.CH<sub>2</sub>.CHO) as an assistant for mordanting wool and woolen fabrics in connection with salts of chromic acid.

The application of many dyestuffs to textile fibers requires the use of a mordant. In the case of dyeing operations on wool, the mordant frequently is applied before the dyestuff and usually takes the form of a metallic salt, such as a chromate or a dichromate, fixed in the wool fibers. Salts of chromic acid are the principal mordants which are used to any extent, but salts of other metallic elements such as aluminum, iron, tin and similar metals, that is, salts of aluminic, ferric, stannic, etc. acids as well as of chromic acid, have been proposed for this purpose and my invention is applicable thereto in so far as their use is analogous to that of the salts of chromic acid. The dyeing of silk and other animal textile fibers may closely follow, in certain instances, the methods applied to wool. I shall hereinafter describe my invention with respect to mordanting operations on wool employing a salt of chromic acid as the mordant, but the invention is not limited to this application.

Many substances have been employed as mordanting assistants. These were, for the most part, acidic substances both organic and inorganic. Among such assistants may be listed sulphurous and sulphuric acid and their salts, oxalic, acetic, lactic and tartaric acids and various compounds of these latter substances. In the employment of acidic assistants with chromic salts, it is generally true that the rate at which the chromic salt is absorbed in the fibers varies directly with the acidic strength of the assistant, and that in cases where the absorption is rapid the tendency of the dye subsequently fixed on the fiber to rub off is increased. This tendency is technically known as "crocking". Aldol possesses an advantage due to the fact that it causes a gradual and even deposition or reduction of the mordant at a slower rate

than acidic assistants. It produces dyeings that are exceptionally level and which have much less tendency to "crock" than any of the assistants heretofore employed.

I may practice my invention by treating woolen fibers or fabric in a boiling bath comprising a solution of sodium dichromate and aldol. The amount of aldol employed may very widely according to the dye being used. In general, the quantity ranges from about one-third of the molecular proportion of sodium dichromate which is present to an amount slightly in excess of the molecular proportion of sodium dichromate. The action of the aldol effectively fixes the chromium salt, probably as a complex hydrate, in the woolen fibers. The fabric may now be removed from the bath and rinsed preparatory to being dyed.

The following example is illustrative of the invention as applied to the usual practice of mordanting woolen fabrics:

A bath is prepared which contains 3% of sodium dichromate and to this is added 3% of a 50% solution of aldol. The bath is heated to 120° F. and the cloth is entered into the bath. The bath is then slowly brought to boiling temperature and boiled for an hour. At the end of this time the cloth is removed, rinsed, and entered into the dye bath proper which is heated to 120° F. This dye bath contains 3% of Chrome blue black R (color Index No. 202) and 1.5% of gallocyanine (color Index No. 883). It is slowly brought to a boil and boiled for an hour or until the dyestuff is exhausted. The cloth is then rinsed and finished in the usual manner.

In industrial practice the above procedure is frequently varied. Instead of first subjecting the textile fibers to a mordanting bath and then to a dyeing bath, the fibers are dyed and the mordant is then affixed in the same or in a separate bath. This process is termed the "after-chrome" or "top-chrome" process. When it is used it is customary to employ about one-half as much mordant as is used when the mordant is applied first. Assistants are not always desirable in top-chrome dyeing, their use being dependent upon the type of dye used. I have found that aldol is

particularly valuable, producing excellent results, as an assistant in "top-chrome" processes with dyes of the chromotrop series, of which Chromotrop F 4 B color Index No. 5 180) is a typical member.

The method of practicing my invention will be apparent from the foregoing description. Many variations in manipulation will be required by different conditions and are 10 included within the scope of the invention.

I claim:

1. An assistant for mordanting with salts of chromic, aluminic, ferric and stannic acids which comprises a substantial proportion of 15 aldol.

2. An assistant for mordanting animal textile fibers with salts of chromic acid which comprises a substantial proportion of aldol.

3. An assistant for mordanting animal 20 textile fibers with alkaline metal dichromates which comprises a substantial proportion of aldol.

4. A process for mordanting wool which comprises treating the wool with a solution 25 containing a salt of chromic acid and a substantial proportion of aldol.

5. A process for mordanting wool which comprises treating the wool with a solution containing an alkaline metal dichromate and 30 a substantial proportion of aldol.

6. A process for mordanting wool which comprises treating the wool with a solution containing sodium dichromate and a substantial proportion of aldol.

35 7. A process for mordanting wool which comprises entering woolen cloth into a bath containing 3% sodium dichromate and 3% of a 50% solution of aldol at a temperature of about 120° F., heating the bath to boiling 40 temperature and continuing to boil the bath for a period sufficient to affix the chrome mordant in the fibers of the cloth.

8. A process for top-chroming wool which 45 comprises subjecting the wool to the dyeing action of a dyestuff of the chromotrop series and then treating it with a solution containing a salt of chromic acid and a substantial proportion of aldol.

50 9. A process for top-chroming wool which comprises subjecting the wool to the dyeing action of a dyestuff of the chromotrop series and then treating it with a solution containing sodium dichromate and a substantial proportion of aldol.

55 10. A process for mordanting wool which comprises entering the wool into a bath containing sodium dichromate and a quantity of aldol equal to from about one-third to slightly in excess of the molecular proportion 60 of sodium dichromate in the bath, and thereafter heating the bath to boiling for a period sufficient to affix the mordant in the fibers of the wool.

65 11. A process for mordanting wool which comprises entering woolen cloth into a bath

heated to about 120° F. and containing sodium dichromate and a quantity of aldol equal to from about one-third to slightly in excess of the molecular proportion of sodium dichromate in the bath, and thereafter heating 70 the bath to boiling for a period sufficient to affix the mordant in the fibers of the wool.

In testimony whereof, I affix my signature.

ALAN A. CLAFLIN.

75

80

85

90

95

100

105

110

115

120

125

130